

June 7, 1927.

1,631,173

H. F. WEISS

WALL BOARD AND PROCESS OF MAKING THE SAME

Filed Aug. 22, 1921



INVENTOR

Howard F. Weiss

BY  
Pennie Davis Brown & Edwards

ATTORNEY

Patented June 7, 1927.

1,631,173

## UNITED STATES PATENT OFFICE.

HOWARD F. WEISS, OF MADISON, WISCONSIN, ASSIGNOR, BY MESNE ASSIGNMENTS, TO  
WOOD CONVERSION COMPANY, OF CLOQUET, MINNESOTA, A CORPORATION OF DEL-  
AWARE.

### WALL BOARD AND PROCESS OF MAKING THE SAME.

Application filed August 22, 1921. Serial No. 494,150.

There are now on the market three general types of wall board made from wood. The first type is made as follows: Round wood is ground into a mechanical pulp on 5 grinding equipment such as is used in making ordinary ground wood pulp for paper manufacture. To this ground wood pulp is added a certain amount of chemical pulp to give added strength to the finished product, 10 then the mixture is flowed over an ordinary board machine into a sheet of paper having the thickness of ordinary card-board. At the end of the paper making machine the sheets are wound into rolls of a size convenient for transportation. The wall board is made from them by un-rolling five rolls or more simultaneously and gluing or cementing the various sheets of paper together, 15 usually with an adhesive such as sodium silicate. The sheets of paper or card-board thus glued together are then cut to the desired size and dried and in this form are commercial wall board. Some manufacturers use waste papers in whole or in part 20 instead of ground round wood, but without change in the essentials of the process as above outlined. Wall boards of this type are sold in the United States in greater tonnage than those of any other type.

30 A second type of wall board now on the market is made by grinding the wood to a pulp and then beating the pulp in standard paper making beaters and finally flowing it into trays; these trays are then put into a 35 hydraulic press and the mass is compressed into a dense product which is then removed from the press, dried, trimmed, and surfaced. Chemical pulp can be substituted in whole or in part for ground wood pulp in 40 this type of board. This board consists of but one layer, and usually is denser and has a more compact surface than wall board made from paper sheets.

A third type of wall board is made by gluing 45 or cementing between two heavy sheets of paper, slats of wood placed side by side. This board is expensive because of the cost of the wood slats and because of the relatively large quantity of sodium silicate or 50 other adhesive that must be used in holding the slats together and in fastening the covering sheets firmly to the wood. The

covering sheets are relatively tough and thick and have the characteristic appearance and surface texture of paper. 55

These three types include all of the various varieties of wood wall board now on the market in a large way. They all involve the step of first preparing a wood pulp either mechanically or chemically in standard pulp 60 making equipment. Such equipment is, from its very character, expensive to install and expensive to operate, and requires large floor area, particularly for the driers of the paper making machine. Furthermore, the manufacture of all of these types starts with logs 65 of good size and quality, which, if not used in the manufacture of wall board, could well be used in the manufacture of newsprint paper and even more expensive papers. An 70 aside from the standard pulp-making equipment used in these processes, the boards themselves are made on large and expensive machines requiring large floor area; the single exception being the one ply board 75 made on a press as above outlined.

All of the wall boards above described rely mainly for their strength upon the interlacing and interlocking of the fibers and, therefore, their processes of manufacture aim to 80 make a pulp having fibers as long as possible. In general, for best results, this requires the use of round wood of good quality and of grinding equipment well designed and carefully maintained. But around 85 every saw mill there accumulates large quantities of what may be termed saw mill offal or wood waste, such as slabs, edgings, trimmings, sawdust, shavings, and bark. Some of this material such as the slabs and edgings, is marketable, under favorable shipping conditions, to paper mills, but though the quality of fiber in the slabs and edgings is as good or better than the general run of fiber from round wood, the pieces of wood 90 are in such physical condition that they are not readily reduced to a pulp, with the result that the yield of fiber is low, the quality of the pulp is poor, and the practical difficulties of operation are enormous. 95

Also, around every saw mill there accumulates large quantities of decayed wood. Some of this is usually saw mill offal or wood waste such as slabs, edgings and trim-

nings for which there has been no market and, continued exposure of which to the elements has resulted in decay of the wood. Some of the rotted wood is usually from the hearts of overripe trees or from lumber piles not properly protected. In general, the rotting or decay of wood is the result of the action of fungi which attack the lignin components of the wood by a process of oxidation whereby the lignin is largely converted into a gas and so passes off into the atmosphere. The usual fungi do not attack the cellulose constituent of the wood and do not attack the resin components to any appreciable extent.

There is a small market for decayed boards, not for building purposes, but as a facing for the surface of the ground when ore is to be piled up; but in accordance with my present invention, such inferior lumber can be put to better use and I can even use wood that has so far decayed as to have substantially no mechanical strength. For instance, I can make use of the hearts of logs that are so far oxidized by the fungi that the wood falls apart and has to be swept up with a broom. Such material is not as good for my purpose as sound wood, but there are some advantages resulting from its relatively high cellulose content and its relatively high resin content. The power consumption necessary for putting this rotted wood into proper condition for use in accordance with the present invention is of course relatively low because of the physical weakness of the material.

Any wall board process that depends for its raw material on grinding round wood on a stone requires the expenditure of large quantities of power. For example, a ton of ground wood pulp, suitable for making the plies of a wall board, requires 1200 to 2400 horsepower hours for grinding alone. This great quantity of power is consumed, partly in the mechanical work of tearing the fibers one from another, but more largely in frictional loss at the surface of the stone where it rubs with heavy pressure on the log of wood and where the log acts as a brake on the stone. This frictional loss is dissipated in the form of heat and the heat is carried away in the cooling water and thus is lost. The cooling water, after separation of the fibers, is ordinarily run to waste.

It is an object of the present invention to provide a ready market for saw mill offal or wood waste, including decayed wood.

It is a further object of the present invention to produce a wall board consisting essentially of a single ply, this board preferably being free from sodium silicate and being uniform throughout. The board may have a surface that is dense and capable of taking a good finish and even a high polish, and if desired can be ornamented by grain-

ing and painting methods now well developed in the decoration of sheet material such, for instance, as sheet metal.

It is a further object of the present invention to produce a wall board of acceptable character from saw mill offal such as slabs, trimmings, edgings, sawdust, shavings and even bark and decayed wood, and to do this with a power consumption far below that ordinarily needed and in machinery and buildings less expensive than those now needed for the production of wall board from ground wood or from chemical pulp. Other objects and advantages of the present invention will become clear from the following description which is to be taken in conjunction with the accompanying drawings, wherein:

Figure 1 is a diagrammatic representation, in elevation, of a complete plant for making wall board by the present process, and Fig. 2 is a diagrammatic plan view of the same.

The wall board of the present invention comprises a binder and a filler and the novelty in the product lies particularly in the binder and in its combination with a filler of special character. There is also novelty in the process of making and using the binder, particularly for the manufacture of a wall board such as that hereinafter described.

The binder consists essentially of lignocellulose gelatinized by mechanical disintegration preferably in the presence of water and preferably with the aid of a gelatinizing chemical such as caustic soda. This binder per se when dried is a hard and horny mass having good binding qualities and yet offering no impediments to usual wood working operations such as sawing, planing, chiseling, and the like. The binder can be made from sawdust or somewhat larger particles of raw wood and preferably is made by crushing or rolling the wood particles between relatively rotating discs whereby the fibers are torn apart and subjected to pressure in the presence of water and ultimately are converted in part at least into a gelatinized mass. If wood particles other than sawdust are used as the raw material for the binder, they are preferably obtained by chipping, hogging or shredding mill waste or offal or decayed wood, and not by grinding solid wood on a stone as in pulp making. As a step in the gelatinization or partial gelatinization of the sawdust or similar wood particles, a water-logging procedure is applied to the particles to facilitate their mechanical disintegration and conversion into gelatinous material. Preferably this water-logging operation is applied to the wood after it has been reduced to a fineness comparable to that of sawdust, or even finer than this.

The filler need not be separate fibers, as

excellent results are had by using bundles of fibers such as sawdust preferably screened to take out the finest and the coarsest particles. Incompletely gelatinized wood particles can constitute the filler and, as herein-after pointed out at length, there are many practical advantages in using sawdust or equivalent fibrous structures wherein the fibers are grouped together or aggregated as in the living tree, and wherein these fiber aggregates have been gelatinized to some extent on their exposed surfaces by passing them between the relatively rotating discs of the crushing or rolling apparatus.

15 The details of the process and of the product in their preferred embodiment will be better understood from the following disclosure.

*The binder.*

20 Starting with saw mill offal or waste, such as slabs, edgings, trimmings, shavings, and even bark or decayed wood of whatever origin, or with mixtures of these, or starting 25 with paper mill offal or waste such as crooked bolts, or limbs or branches such as are commonly left in the forest, either with or without preliminary removal of the bark by usual methods, as in the so-called drum 30 barker, I pass the waste through a "hog" such as is used at saw mills for cutting up waste wood to make it suitable for fuel, or through a "chipper", such as is used in preparing wood for the soda, sulfite or sulfate 35 process, or through a "coarse shredder", such as is sometimes used at saw mills in place of a hog to reduce wood to small chips or fragments. If desired, a hog and a shredder may be used in conjunction, the hog cutting the 40 wood into fragments say two inches long, and the shredder beating these fragments into smaller pieces. Good sound round wood can of course be used as raw material but mill waste is much cheaper and is entirely 45 satisfactory. All of these operations which, for lack of a better name, I will hereinafter designate as "chipping", are carried out by a cutting action which requires very much less power than if the waste were reduced to a 50 pulp by holding solid blocks of it against a rapidly rotating stone as in grinding wood for ground wood pulp. Also, the product resulting from chipping is entirely different 55 from ground wood pulp.

55 Thus, by chipping, the saw mill or paper mill offal is reduced to a mass of chips or wood particles of a size about one-half inch in length by one-eighth inch in diameter, or less. If the mill waste is all in the form of sawdust, or other like small particles, the chipping and shredding steps can be omitted.

60 These small wood particles (which, as above explained, may be nothing more than sawdust or may be larger particles), are next passed into hopper 2 (Fig. 1) prepara-

tory to delivery into a machine 3 whereby they are torn apart and reduced in part, but preferably not entirely to separate fibers. The machine 3 for separating the fibers may be constructed in many ways but best results 70 have been obtained by me in an apparatus having two discs of metal, one of which is rotatable with respect to the other and between which the sawdust or other relatively small wood particles are subjected to a rolling action to tear, or more strictly speaking, crush the fibers one from another. Good results have been obtained by the use of disc grinders commonly known as "corn cracklers" of which the 36" single disc mill 80 of Bauer Bros. Company, Springfield, Ohio, U. S. A., is a good illustration. The details of such a disc grinder or corn cracker are well illustrated in U. S. Patents Nos. 565,690 and 817,610. In such a machine the action 85 of tearing the wood fibers apart resembles somewhat the disintegrating effect of rolling a wooden match under foot on the floor, excepting, however, that because of the relative rotative movement of the discs, each 90 piece of wood or bundle of fibers has a gyroscopic motion about the axis of the rotating disc so that not only are the fibers and bundles of fibers subjected to a crushing action, but they are subjected to a twisting 95 effect. As one disc rotates with respect to the other, the small wood particles or bundles of fibers will naturally take up positions along radii of the rotating disc and, since their outer ends travel through a 100 greater distance than their inner ends, there will be a decided tendency for the fibers to slip longitudinally with a twisting movement. That is to say, there is not only a crushing pressure perpendicular to the axes 105 of the individual fibers, but there is a strain, in shear, superimposed on the crushing strain and parallel to the axes of the fibers, or more strictly speaking, radial to the rotating plate of the machine. It will be understood that the two plates of the machine 110 between which the particles are rolled have slightly concaved faces and can be roughened or surfaced to accelerate the disintegrating action or fiber liberation. Both 115 plates may rotate in opposite directions; or one may be stationary and the other rotatable. The working faces of the discs are preferably of metal; but of whatever material, the surfaces are adjusted in such manner that they do not touch. It is also important that means be provided for adjusting the distance between the plates in accordance with the size, character and origin 120 of the wood particles under treatment, and the character of the product desired. It is a rolling and twisting action rather than a grinding action that gives best results in the manufacture of the products hereinabove described. Too much of the grinding 125

action produces too large a percentage of wood flour, as distinguished from fiber pulp.

The power consumed for reducing wood to pulp by first chipping, then shredding and then rolling the small wood particles between two relatively moving discs, as above described, is much less than that required for tearing the fibers apart on an ordinary paper mill grindstone; for not only has the chipping and shredding cut the fibers from the solid wood, but the disintegrating or fiber liberating power has been applied to the particles in compression and in shear, and therefore along their lines of least resistance. Also, in this process, friction and frictional losses have been reduced to a minimum. The bundles of fibers act as rollers between the moving surfaces while rolling one upon the other. No water need be added at this stage.

To reduce the wood to the desired condition, it may be passed repeatedly through the same fiber liberating machine. Or, if desired, a series of fiber liberating machines may be used in each succeeding one of which the relatively moving surfaces are so adjusted as to give best disintegrating action on the partially reduced wood with which it is supplied. The latter procedure is preferable and passage through three of the grinders will disintegrate the sawdust or similar wood particles to the extent desired at this stage of the process.

A suitable arrangement of the three grinders is indicated diagrammatically in Fig. 2 of the drawing, where the material delivered from disc grinder 3 to box 4 is carried by an elevator 5 to a hopper 6 adapted to deliver to a disc grinder 7. When delivered from the latter to box 8, the mass can be lifted by either of conveyors 9 or 10 and delivered to the hopper of grinders 11 or 12, which in turn deliver to tank 13 from which the mass ultimately can be conveyed to other disc grinders of the series.

The next step consists in conveying the finely divided wood from storage tank 13 to a tank 14 where a water-logging procedure is initiated. This water-logging is used because wood that is wet is very much weaker and can be torn apart with less expenditure of energy than wood that is dry—the fibers separate from one another more easily. For example, wet wood has, in compression, about one-half to one-third of the strength of dry wood. This water-logging can be done conveniently by first submerging the fiber aggregates in water heated nearly or preferably to the boiling point, and then, while the wood particles are submerged in a closed tank, subjecting the mass to pressure, such as steam pressure, to force the hot water into the fiber aggregates.

As an alternative procedure, the fiber aggregates can be thoroughly heated in the

hot water and then, while the temperature of the water is near or at the boiling point, cold water can be added to cause contraction of the expanded air and gases of the wood particles, thereby drawing water into the pores or voids of the particles.

As another procedure, the fiber aggregates while hot from the exposure to hot water can be dumped into cold water to cause contraction of the expanded air and gases, as above described. Under some circumstances it is more economical merely to let the hot water and the submerged wood particles cool by radiation, for by so doing, large quantities of water will be drawn into the pores and voids of the wood.

By such a treatment fiber aggregates (such as sawdust or chips that have been mechanically disintegrated in the three grinders) can be so thoroughly saturated with water that they will sink in water in an hour or less. If they were merely submerged in water, it would take months and, in the case of resistant woods, years, before the fiber aggregates soaked up enough water to sink. The heating in hot water is not intended to be a cooking operation and there need be no chemical present to effect cooking. Nevertheless, the hot water dissolves out some or perhaps all of the highly soluble constituents of the wood. When western larch is used as the wood, this is a valuable feature of the process because of the possibility of recovering valuable sugar making ingredients from the liquor.

As an alternative and the preferred procedure, the water is hot and contains 1% of caustic soda (NaOH) by weight, and the fiber aggregates are soaked in this liquor at boiling temperature and at atmospheric pressure for about one hour, after which the fiber aggregates are dumped into a second tank containing caustic soda solution of the same strength but at room temperature. These operations can be carried out in tanks 14 and 15 where 14 is the hot soda tank and 15 is the cold soda tank. The presence of soda facilitates the penetration of moisture into the fiber aggregates and in addition is a component useful in subsequent steps of the process.

From tank 15 the cold and water-logged fiber aggregates, together with the soda liquor, are delivered to a press 16 for the removal and recovery of the caustic soda liquor. This recovered liquor is returned to one of the soda tanks and is used over again. This press may be of the roller type such as was commonly used for squeezing the liquor from malt sprouts in the beer industry. This moist mass of water-logged fiber aggregates, impregnated with a small quantity of caustic soda, is next delivered to a hopper 17, and from there passes into a second series of grinders similar in structure to those

above described, but with their plates closer together. The soda content will then be about 40 lbs. per ton of fiber aggregates, by dry weight. Caustic potash can be used as a 5 substitute for caustic soda.

The fiber aggregates are delivered from hopper 17 to the grinding mill 18. Water is passed through the mill with the fiber aggregates. This water can be supplied conveniently by means of a pipe 19 which delivers a steady stream into the top of hopper 17. The use of water in the mill is to facilitate the flow or flushing out of the material and not because of the cooling action 10 of the water. In fact hot water can best be used for this purpose, because of its effect in lowering the resistance of the wood to the crushing action and similar disintegrating stresses. No caustic soda or other 15 chemical need be added to the water for the fiber aggregates have already been charged with enough of the caustic soda to insure the results desired.

The pulpy mass delivered by grinder 18 is lifted by a pump 20 to a second grinder 21 where the disintegrating treatment is repeated. Ordinarily three of these grinders are sufficient to produce the effect desired, though more than that number can be used 20 when more complete chemical and physical changes of the wood are deemed advisable.

As the wood proceeds through this series of grinders the particles or fiber aggregates are torn apart to yield separated individual 25 fibers and, furthermore, these fibers undergo a chemical change and ultimately are delivered from the last grinder of the series into storage tank 22 in a gelatinous structureless form well adapted for use as a binder 30 in the wall board of my present invention. But with the individual fibers so separated and gelatinized, there is mixed a relatively high percentage of fiber aggregates that have resisted complete physical disintegration and 35 are gelatinized only on the surface.

It is well recognized in the literature that the hydration qualities of lignocellulose or wood are not very great and that mechanical wood pulp suffers little alteration by beating 40 in a paper maker's beater. But I have found that when lignocellulose or wood is crushed or rolled under pressure in a corn cracker and in the presence of water, hydration will begin even with the first mill of 45 the series and the hydration will progressively increase as the wood is reduced to fiber and the fibers are broken and crumbled under pressure. The water-logging treatment to which the wood has been subjected 50 and the addition to it of a small quantity of caustic soda both facilitate hydration. However, it is entirely possible to produce a gelatinized lignocellulose without giving it the water-logging treatment and by merely rolling 55 and breaking the fibers in cold water.

While the hydration or gelatinizing effect may not be very great in grinder 18 (Fig. 2), the other and particularly the last grinders of the series in which the plates are set close together, so completely comb 70 out, crush, and gelatinize the fiber aggregates that the fibrous structure of a large proportion of the separated fibers disappears entirely.

As above explained, the resultant product 75 is a slimy mass of lignocellulose consisting in part of gelatinized fibers and in part of undisintegrated and superficially gelatinized fiber aggregates. The gelatinized lignocellulose might perhaps be called "hydrated 80 lignocellulose", though I know of no method for determining how many water molecules have attached themselves to the cellulose molecule, or if indeed any such water molecules have been added. I know that the 85 chemical structure of the gelatinized material must be different from that of lignocellulose, and as appears below, the physical structure is likewise radically different. Therefore, for lack of a better name, I have 90 herein designated this material, which is to be the binder or binding element of the wall board, as "gelatinized lignocellulose". Gelatinized lignocellulose, as the term is herein used, means wood fibers (lignocellulose) 95 that have been so treated mechanically as to be completely torn and broken so that their length is but a fractional part of their original length, say, for instance, one-tenth or less; furthermore, the original wood 100 cellulose has been changed chemically and perhaps to the extent of adding to it an unknown number of water molecules. The gelatinous component of the material delivered from the last grinder, when wet, is a 105 slimy mass which on drying shrinks enormously and is inclined to warp and forms a dense, hard, bone-like mass of considerable strength and without appreciable fibrous structure, but inclined to split or flake and 110 of a color usually somewhat darker than that of the wood from which it was made. Made from pine, spruce or hemlock the material is cream colored, and made from fir, tamarack or larch it is somewhat darker in color. 115 It can be made readily from any of these woods and others, but with cedar the problem is more difficult because of difficulties in chemically changing the water-resistant fibers of such gymnosperms.

Both physically and chemically, gelatinized lignocellulose is readily distinguishable from wood flour, though according to my experiments, wood flour often results from prolonged mechanical treatment of wood fiber, as, for instance, when the fiber is passed repeatedly through a Jordan. The pulpy mass of partially gelatinized lignocellulose delivered by the last grinder of 125 this series is the material used by me for 130

the production of wall board in accordance with the present invention. The gelatinized component of this lignocellulose mass not only constitutes an appreciable percentage 5 of the total material used, but acts as a binder to unite with and hold in place the other and more inert material or materials with which it is associated. These other materials properly may be designated as the 10 filler.

A feature which readily may be incorporated in the above described process of making gelatinized lignocellulose is the recirculation of the water in some, at least, of the 15 fiber-liberating machines which, with the soluble material in the wood, can be recovered in a manner similar to that described in my U. S. Patent No. 1,339,489, issued May 11, 1920. Furthermore, whenever a plurality 20 of fiber-liberating machines are used in series to progressively reduce the wood particles to pulp, and then to gelatinize the pulp, the circulation of the water to take out soluble material (as from western larch), can be on 25 the counter-current principle, that is to say, the water used in the last machine or grinder of the series can be filtered off from the pulpy material delivered therefrom and can be introduced as the flushing water of the 30 machine next preceding, and so on throughout the series, the strongest solution of soluble constituents being drawn off from the partially disintegrated shredded wood particles of the machine into which these particles 35 initially were delivered.

#### *The filler.*

When the pulpy mass is delivered from the last grinder it consists, as above explained, of gelatinous lignocellulose, adapted 40 to serve as the binder of the wall board, and other material somewhat like sawdust but more finely divided, and with the component particles gelatinized on the surface. I have 45 called these small wood particles "fiber aggregates" and by fiber aggregates I mean five or more wood fibers still joined together as in the living tree. The fibers need not, however, be of full length and ordinarily are 50 not.

The relative proportions of the two ingredients of the mixture may be varied through 55 relatively wide limits. Up to a certain point the larger the percentage of gelatinized lignocellulose the stronger is the resultant board. The board should contain 25% or more by dry wood weight of the gelatinized lignocellulose and 30% or more by dry wood 60 weight of fiber aggregates. A mixture composed of 60% gelatinized lignocellulose and 40% fiber aggregates by dry wood weight to which enough water has been added to make the mass flow readily gives a very strong, stiff and satisfactory wall board. 65 Spruce or pine give a stronger board than

cedar but any one of these woods or mixtures of any of them are suitable.

#### *The sizing.*

While the pulpy mass is being mechanically disintegrated in grinders 18, 21 and succeeding grinders, there preferably is added to it a solution of sodium resinate in water, and after this has been thoroughly mixed with the mass and ground into it, a 70 water solution of alum is introduced (as at the last grinder) to convert the soluble sodium resinate into an insoluble resinate. This treatment sizes the fiber aggregates, and also sizes the gelatinized lignocellulose, and 75 makes them and the finished board highly 80 resistant to moisture. The sizing is uniform throughout the entire board. These sizing materials may be omitted entirely when waterproofing is not desired without injuring 85 the strength or other characteristics of the board, excepting that of its resistance to water. Normally the percentage of sodium resinate may be from two to eight per cent of the dry weights of the other components, depending 90 on the amount of wood used and particularly its resinous content and the degree of waterproofing desired in the finished product. When decayed wood is being used in appreciable quantity, this wood, if of a 95 coniferous variety, may be abnormally high in its percentage of resin, and under these conditions due allowance must be made in the percentage of resinate added to the pulp. The quantity of alum is in proportion to the 100 sodium resinate, due allowance being made for the amount of water present, etc.

If a fireproof board is desired, the requisite amount of ammonium sulfate or analogous fire retardant can be added to the 105 batch and uniformly ground into it while it is passing through this series of grinders.

A non-mineral coloring, such as an aniline dye, can also be added if a colored board is desired. This is particularly advantageous 110 when the board is to be finished in imitation of mahogany.

#### *Pressing.*

The now thoroughly mixed mass of sized 115 gelatinized lignocellulose and wood fiber aggregates is next delivered to a flow box 23 (Fig. 2) like those in ordinary paper making machines, and so constructed as to maintain a constant head in the box with an 120 overflow through pipe 24 into the underground storage tank 22 (Fig. 1). A constant stream of the pulpy mass flows out of a horizontal slot in the side of the box under a gate 25. This gate is provided with 125 a rack and pinion 26 by which it may be raised or lowered to vary the size of the stream. As the thick mixture flows through the slot it is delivered in a uniformly thick 130 layer on a traveling wire screen or conveyor

27 which is mounted on cylinders 28 and 29, and is supported along its upper stretch by power-driven rollers 30. This prevents sagging of the screen or conveyor while its load of material is being delivered to and from the press. To make a board about  $\frac{3}{16}$ " thick, the thickness of this layer as it flows onto the wire conveyor is approximately  $2\frac{1}{2}$ ".

10 The width of the wire screen conveyor or belt corresponds with the length of the board or panel to be made, and the cellulosic mass is prevented from flowing off the sides of the conveyor by means of two stationary 15 baffles 31 (Fig. 2). These baffles are adjustable laterally to accommodate several widths of cellulosic mass to accord with changes in the length of the boards to be made. In general, a board length of 16 feet is suitable 20 for ordinary trade demands. Converging boards 32 smooth off the top of the pulp layer. Thus the cellulosic mass in a relatively thick and uniform layer 16 feet wide and  $2\frac{1}{2}$  inches thick on the wire screen conveyor is carried forward between the stationary baffles 31 and ultimately passes between the platens of a powerful press. The wire screen conveyor moves forward with an intermittent movement and as soon as the 25 proper amount of the mass is between the platens a rectangular die 33, having inside dimensions corresponding to the size of the board to be made, is lowered into the mass until it rests on the wire screen conveyor. 30 The cellulosic mass is so fluid that it readily moves aside to permit this lowering of the die. Then the upper platen, which fits within the die with a substantially water-tight joint, is lowered into the die and compresses 35 the cellulosic mass, while simultaneously squeezing its excess water both upward and downward through suitable slots in the platens. It is advantageous to apply suction to these openings in the top and bottom 40 platens to facilitate prompt removal of the water. Much of the water drips out of the mass while it is on the wire screen and before it reaches the press, but the proportion remaining should be reduced by pressure 45 and suction to about 60% of the total weight of the compressed board. A pressure of 200 lbs. per square inch applied gradually over a period of half a minute and left on for a period of five to ten seconds 50 will, when supplemented by adequate suction, effect the desired extraction. The liquor thus drawn from the pulpy mass is not thrown away but, on the contrary, is fed back into the last series of grinders, thereby economizing in water and conserving 55 whatever binding agents and other soluble components of value may have passed into the water. As soon as the compressing is completed, the suction is cut off and air under pressure is applied in place of the suc-

tion. The platens then separate, the compressed air releases the board from the platens, the die lifts, and the wire screen conveyor moves forward until a fresh amount of material has passed between the platens when the operation just described is repeated. This operation is done mechanically and takes less time than a minute to press each sheet.

#### Drying.

The compressed cellulosic mass is carried forward from the press on the wire screen conveyor or belt and when picked up from this belt by a suction plate 34 is in the form of a damp, fairly stiff, compressed sheet. Suction plate 34 is adjustable vertically in supports 35 to transfer the compressed sheet vertically and sidewise into a dry kiln 36. This kiln may be of the tunnel type heated by steam coils and provided with well known means for regulating the circulation of air, its humidity, temperature, etc., to secure most effective and uniform drying action, and to lessen such tendency as there may be for warpage of the boards. The dry kiln removes the water from the boards so that they emerge from the kiln dry, stiff and hard.

#### Finishing.

The boards are next run through saws and cut to desired size or shape and in that form are marketable in place of wall board made by usual processes. The boards may be 100 nailed directly to the studding of a building to serve in place of lath and plaster, and like wall board now on the market, may be sawed and similarly cut to meet the needs of the builder. But unlike wall boards of more usual manufacture, they contain no sodium silicate or other mineral harmful to the saws and other edge tools of the carpenter. On the contrary, they consist throughout of 105 nothing but woody material through which a saw or chisel will work as readily as through solid wood and with no more injury to the edge of the tool. The resin size and the ammonium sulfate, if present, are not 110 harmful to edge tools.

Such small amount of caustic soda as remains with the cellulosic material after squeezing of the mass at press 16 is neutralized by the alum and gives to the product 115 no objectionable characteristics.

In many respects this new product is different from wall board made from paper sheets cemented together, for, if desired, the wall board of the present invention may be 120 passed through an ordinary wood planer to finish the surface, or through a sand machine to dress its surface, or between steel rolls to give the surface either a high polish or to impress in or on the surface patterns or 125 designs or to give a finish similar to burlap 130

or canvas. Likewise, the finished and even polished face of the board may be treated much as sheet steel is now treated to give it the appearance of grained mahogany or 5 other woods. The surface can be painted and decorated much as can be done with solid wood, excepting that it has not the characteristic grain of wood, but on the contrary, if made with fiber aggregates, has a 10 uniform and pleasing mottled appearance not unlike the so-called oatmeal wall papers.

As above indicated, the process by which 15 this novel and valuable product is made, may vary in many of its details, both as to the origin of the raw materials and as to the procedure by which these materials are treated to bring them into proper physical and chemical condition to unite under pressure and kiln drying into the product described in detail above. It is of particular 20 importance, however, that no chemical need be used in the process and that water alone, together with suitable mechanical manipulations, such as cutting, rolling, and twisting, 25 properly repeated, is sufficient to convert saw mill offal such as slabs, edgings, trimmings, sawdust, shavings and even bark, into a readily marketable product and with relatively low power consumption.

30 The apparatus whereby the process is carried out obviously may vary in details without fundamentally altering either the process or the product claimed herein. Novel features of the apparatus will be claimed in 35 a separate application. The present application describes further developments in the invention described and claimed in my co-pending application, Serial No. 470,967, filed May 19, 1921.

40 I claim:—

1. The method of preparing a wall board binder, which consists in chipping saw mill offal, crushing and rolling the chips until reduced to small particles and then water-logging said particles, and mechanically disintegrating the water-logged particles while wet until at least 25% of the mass by dry wood weight has been reduced to a structureless, gelatinous mass, substantially as 50 described.

2. The method of preparing a wall board binder, which consists in chipping saw mill offal, repeatedly crushing and rolling the chips until reduced to small particles, then water-logging said particles, and repeatedly crushing and rolling the water-logged particles between relatively rotating discs, substantially as described.

3. The method of preparing gelatinous 60 lignocellulose, which consists in chipping saw mill offal, repeatedly crushing and rolling the chips while dry until reduced to small particles, water-logging said particles, and then repeatedly crushing and rolling said 65 water-logged particles between relatively ro-

tating discs until converted into gelatinous lignocellulose to the extent desired, substantially as described.

4. The method of preparing a wall board binder, which comprises chipping saw mill 70 offal, reducing the chips to small wood particles by repeatedly crushing and rolling the chips while dry, water-logging said small particles and mechanically disintegrating the water-logged particles in water until at least 75 25% of the fibers have been crushed and broken and converted into a structureless gelatinous mass.

5. The method of making wall board, 80 which consists in mechanically disintegrating small wood particles to form a mass consisting of about 50% gelatinous lignocellulose and 50% of fiber aggregates by dry wood weight, shaping and pressing into a board and drying and finishing the board, 85 substantially as described.

6. The method of making wall board, 90 which consists in water-logging small wood particles, crushing and rolling said particles while wet until converted into gelatinous ligno-cellulose to the extent of more than 25% and less than 70% by dry wood weight, shaping and pressing into a board and drying and finishing the board, substantially as 95 described.

7. The method of making wall board, 100 which consists in reducing saw mill offal to small particles, water-logging said particles by heating in water and then cooling, then mechanically disintegrating said water-logged particles until converted into gelatinous ligno-cellulose to the extent of more than 25% and less than 70% by dry wood weight, flowing the mixture into a layer, pressing said layer into a board and drying and finishing the board, substantially as described. 105

8. The method of making wall board, 110 which consists in chipping saw mill offal, repeatedly crushing and rolling the chips until reduced to small particles, water-logging said particles, then mechanically disintegrating said particles in water until converted into gelatinous ligno-cellulose to the extent of more than 25% and less than 70% by dry wood weight, flowing the mixture 115 into a layer, pressing said layer into a board and drying and finishing the board, substantially as described.

9. The method of making wall board, 120 which consists in reducing saw mill offal to small particles, water-logging said particles, repeatedly crushing and rolling said water-logged particles while wet until converted into gelatinous ligno-cellulose to the extent of more than 25% and less than 70% by dry wood weight, sizing the mixture during said conversion, flowing the mixture into a layer, pressing said layer into a board and drying and finishing the board, substantially 125 as described. 130

10. The method of making wall board, which consists in reducing saw mill offal to small particles, water-logging said particles by heating in water and then cooling, repeatedly crushing and rolling said water-logged particles until converted into gelatinous ligno-cellulose to the extent of more than 25% and less than 70% by dry wood weight, flowing the mixture into a layer, compressing said layer into a board, and drying and finishing the board, substantially as described.

11. The method of making wall board, which consists in reducing saw mill offal to small particles, water-logging said particles by heating in water containing caustic soda and then cooling, pressing to remove and recover the alkaline liquor, then repeatedly crushing and rolling said water-logged particles in water until converted into gelatinous ligno-cellulose to the extent of more than 25% and less than 70% by dry wood weight, flowing the mixture into a layer, compressing said layer into a board, and drying and finishing the board, substantially as described.

12. The method of making wall board, which consists in reducing saw mill offal to small particles, water-logging said particles by heating in water containing about 1% of caustic soda and then cooling, pressing to remove and recover the alkaline liquor, then repeatedly crushing and rolling said water-logged particles in water until converted into gelatinous ligno-cellulose to the extent of more than 25% and less than 70% by dry wood weight, flowing the mixture into a layer, compressing the layer into a board with simultaneous sucking of moisture therefrom, and drying and finishing the board, substantially as described.

13. The method of making wall board, which consists in reducing saw mill offal to small particles, water-logging said particles by boiling them about an hour at atmospheric pressure in water containing about 1% of caustic soda and then cooling, pressing to remove and recover the alkaline liquor, then repeatedly crushing and rolling said water-logged particles in water until converted into gelatinous ligno-cellulose to the extent of more than 25% and less than 70% by dry wood weight, sizing and fire-proofing the mixture during said conversion, flowing the mixture into a layer, compressing said layer into a board with simultaneous sucking of moisture therefrom, and drying and finishing the board, substantially as described.

14. The method of making wall board, which consists in chipping saw mill offal, repeatedly crushing and rolling the chips while dry until reduced to small particles, water-logging said particles, repeatedly crushing and rolling said water-logged par-

ticles in water between relatively rotating discs until converted into gelatinous ligno-cellulose to the extent of more than 25% and less than 70% by dry wood weight, flowing the mixture into a layer, compressing said layer into a board, and drying and finishing the board, substantially as described.

15. The method of making wall board, which consists in chipping saw mill offal, repeatedly crushing and rolling the chips while dry between relatively rotating discs until reduced to small particles, water-logging said particles by heating to about boiling temperature in water containing an alkali and then cooling, pressing to remove and recover the alkaline liquor, then repeatedly crushing and rolling said water-logged particles in water until converted into gelatinous ligno-cellulose to the extent of more than 25% and less than 70% by dry wood weight, flowing the mixture into a layer, compressing said layer into a board, and drying and finishing the board, substantially as described.

16. The method of making wall board, which consists in chipping saw mill offal, repeatedly crushing and rolling the chips while dry until reduced to small particles, water-logging said particles by heating in water containing caustic soda and then cooling, pressing to remove and recover the alkaline liquor, then repeatedly crushing and rolling said water-logged particles in water until converted into gelatinous lignocellulose to the extent of more than 25% and less than 70% by dry wood weight, flowing the mixture into a layer, pressing said layer into a board, and drying and finishing the board, substantially as described.

17. The method of making wall board, which consists in chipping saw mill offal, repeatedly crushing and rolling the chips while dry until reduced to small particles, water-logging said particles by heating in water containing about 1% of caustic soda and then cooling, pressing to remove and recover the alkaline liquor, then repeatedly crushing and rolling said water-logged particles in water until converted into gelatinous lignocellulose to the extent of more than 25% and less than 70% by dry wood weight, flowing the mixture into a layer, pressing said layer into a board, and drying and finishing the board, substantially as described.

18. The method of making wall board, which consists in chipping saw mill offal, repeatedly crushing and rolling the chips while dry until reduced to small particles, water-logging said particles by heating in water containing about 1% of caustic soda and then cooling, pressing to remove and recover the alkaline liquor, then repeatedly crushing and rolling said water-logged particles in water until converted into gelatinous lignocellulose to the extent of more

- than 25% and less than 70% by dry wood weight, sizing and fireproofing the mixture during said conversion, flowing the mixture into a layer, compressing said layer into a board with simultaneous sucking of moisture therefrom, and drying and finishing the board, substantially as described.
19. The method of making wall board, which consists in chipping saw mill offal, repeatedly crushing and rolling the chips while dry until reduced to small particles, water-logging said particles by boiling them about an hour at atmospheric pressure in water containing about 1% of caustic soda and then cooling, pressing to remove and recover the alkaline liquor, then repeatedly crushing and rolling said water-logged particles in water until converted into gelatinous lignocellulose to the extent of more than 25% and less than 70% by dry wood weight, sizing and fireproofing the mixture during said conversion, flowing the mixture into a layer, compressing said layer into a board, with simultaneous sucking of moisture therefrom, and drying and finishing the board, substantially as described.
20. Artificial lumber consisting essentially of a dried gelatinous mass of mechanically disintegrated lignocellulose intermixed with fiber gelatinized on the surface.
21. Artificial lumber consisting essentially of a dried gelatinous mass of mechanically disintegrated lignocellulose intermixed with fiber gelatinized on the surface, a dried gelatinous mass constituting 25% to 70% of the lumber by dry wood weight.
22. Artificial lumber consisting essentially of a dried gelatinous mass of mechanically disintegrated lignocellulose intermixed with fiber gelatinized on the surface, the dried gelatinous mass comprising about 40% of the lumber by dry wood weight.
23. Artificial lumber comprising a dried gelatinous mass of mechanically disintegrated lignocellulose intermixed with fiber aggregates gelatinized on the surface.
24. Artificial lumber comprising a dried

gelatinous mass of mechanically disintegrated lignocellulose intermixed with fiber aggregates gelatinized on the surface, the fiber aggregates constituting about 50% of the lumber by dry wood weight.

25. Artificial lumber consisting essentially of a dried gelatinous mass of mechanically disintegrated lignocellulose intermixed with the residue of mechanically disintegrated and partially gelatinized fiber aggregates.

26. Artificial lumber comprising a dried gelatinous mass of mechanically disintegrated lignocellulose intermixed with a residue of partially gelatinized fiber aggregates, said mass being waterproofed throughout.

27. Artificial lumber comprising a dried gelatinous mass of mechanically disintegrated lignocellulose intermixed with a residue of partially gelatinized fiber aggregates, said mass being fireproofed uniformly throughout.

28. Artificial lumber consisting essentially of a dried gelatinous mass of mechanically disintegrated lignocellulose intermixed with a residue of mechanically disintegrated and partially gelatinized fiber aggregates, said mass being waterproofed and fireproofed uniformly throughout.

29. The method of making wall board which consists in water-logging small wood particles, crushing and rolling said particles while wet to form a mass of about 50% gelatinous lignocellulose and 50% of fiber aggregates by dry wood weight, shaping and pressing into a board and drying and finishing the board, substantially as described.

30. The method of making wall board which consists in mechanically disintegrating small wood particles until converted into gelatinous lignocellulose to the extent of more than 25% and less than 70% by dry wood weight, shaping and pressing into a board and drying and finishing the board substantially as described.

In testimony whereof I affix my signature.

HOWARD F. WEISS.